

# United States Patent [19]

Bigelow

[11] 3,804,632

[45] Apr. 16, 1974

[54] METALLOBORANES AS FOGGING AGENTS  
IN DIRECT POSITIVE EMULSIONS

[75] Inventor: John H. Bigelow, Rochester, N.Y.

[73] Assignee: E. I. du Pont de Nemours and  
Company, Wilmington, Del.

[22] Filed: Feb. 15, 1972

[21] Appl. No.: 226,549

[52] U.S. Cl. .... 96/108

[51] Int. Cl. .... G03c 1/28

[58] Field of Search. .... 96/108, 64

[56] References Cited

UNITED STATES PATENTS

3,655,390 4/1972 Overman .... 96/108

2,717,833 9/1955 Wark ..... 96/108  
3,361,564 1/1968 Bigelow et al. .... 96/64

Primary Examiner—Norman G. Torchin

Assistant Examiner—Won H. Louie, Jr.

[57]

## ABSTRACT

Direct-positive photographic elements having good sensitometric characteristics and aging stability are prepared by incorporating in the silver halide emulsion from  $10^{-8}$  to  $10^{-4}$  mole per 1.5 moles of silver nitrate of at least one metalloborane as a chemical fogging agent selected from the group containing the metals, platinum, nickel, cobalt, rhenium, iron or silver in its structure.

11 Claims, No Drawings

METALLOBORANES AS FOGGING AGENTS IN  
DIRECT POSITIVE EMULSIONS

## BACKGROUND OF THE INVENTION

## 1. Field of Invention

This invention is directed to direct positive colloid silver halide emulsions. More particularly it relates to such emulsions which are prefogged by a chemical fogging agent. Still more particularly this invention relates to direct positive photographic elements comprising a light-sensitive layer coated from such emulsion. In a more particular aspect of the invention, it relates to chemically fogging direct positive emulsions with metalloborane compounds taken from the group consisting of metalloboranes, metallothiaboranes and metallocarboranes. The metalloboranes are borane compounds with metals in which some of the metal atom orbitals (i.e., electron orbits) participate in the icosahedral or other bonding framework.

## 2. Description of the Prior Art

Direct positive emulsions and elements coated therewith are, of course, well known and there are many different methods of producing direct positive images. For example, a silver halide emulsion layer may be given a short overall exposure of high intensity radiation and then given a longer imagewise exposure of lower intensity. Upon development, a direct positive will be obtained. Another method is to expose imagewise and develop and bleach out developed silver and then flash expose and redevelop. A still further method is to use emulsion coated elements, the emulsions of which have been chemically fogged with, for example, formaldehyde, hydrazine, sodium arsenite, silver ions and other nonsulfide fogging agents thus eliminating a solarizing exposure or a bleach out step and redevelopment. Upon imagewise exposure and redevelopment of such chemically fogged elements, a positive image is obtained. In direct positive elements utilizing this latter method there is usually incorporated a desensitizing compound, usually a desensitizing dye. A significant improvement was made in the art by the use of amine boranes as chemical fogging agents in direct positive emulsion systems. Elements comprising such emulsions are described and claimed in Assignee's Bigelow and Burt, U.S. Pat. No. 3,361,564; Burt, U.S. Pat. No. 3,445,235 and Assignee's Overman, U.S. Pat. No. 3,655,390. The Burt patent discloses and claims the use of rhodium and iridium salts in direct positive emulsions described in the above Bigelow and Burt patent and the Overman application discloses the use of bismuth salts as antikink agents. The emulsion coated elements of the above patents are quite fast as compared to direct positive elements of the prior art and avoid many of the disadvantages of long exposure times, low reversal densities, undesirable stain due to desensitizing dyes, as well as undesirable contrast, and a multiplicity of exposure steps and processing operations. Improvements in speed and other sensitometric properties of the above patents are taught by Assignee's Burt, U.S. Pat. No. 3,607,288 issued on Sept. 21, 1971 and Assignee's Burt and Ciavarri, U.S. Pat. No. 3,647,455 issued on Mar. 7, 1972.

The use of a new class of cyclic cage type borane compounds comprising a cage type skeletal framework or a fragment thereof as chemical fogging agents in direct positive emulsion having certain advantages of im-

proved shelf life or aging stability and contrast are described in Assignee's Bigelow, U.S. Pat. No. 3,637,392.

## SUMMARY OF THE INVENTION

It has now been found that the advantages noted in the use of boranes described in the above patents as chemical foggers for direct positive emulsions can be retained by the use of metalloboranes with the added 10 advantage that the compounds have high thermal stability and appear to have moderate resistance to hydrolytic and oxidative degradation thus making them more convenient to use in manufacturing operations. The new metalloborane compounds are selected from the 15 group consisting of metalloboranes, metallothiaboranes and metallocarboranes in which the metal atom orbitals participate in an icosahedral or other bonding framework and are derived from polyhydral or other boranes. They may be added to the emulsions in 20 amounts ranging from  $10^{-8}$  mole to  $10^{-4}$  mole per 1.5 moles of silver nitrate. They may be added to the emulsion as a solution with a suitable solvent, i.e., water, ethyl alcohol, benzene, acetone, dioxane, etc. Dimethyl sulfoxide may also be used for some of the metalloboranes.

Some of the metalloboranes are more effective than others as chemical fogging agents in direct positive silver halide emulsions. Also the effectiveness of some metalloboranes in fogging the silver halide emulsions is 30 not affected by the pH of the system and they show good fogging properties under acid as well as alkaline conditions. It is important, however, that the metalloborane compounds be added at the beginning, during or before the end of the digestion period after the excess salts resulting from the precipitation of silver halides have been removed by washing. The pH of the emulsion is generally adjusted to 9.0 or below. The fogging effect of the metalloboranes is bleachable by light prior to development.

The emulsions of the invention may also contain a rhodium or iridium salt in an amount of from 1.5 to 325 mgm per mole of silver as described in Assignee's Burt U.S. Pat. No. 3,361,564.

Suitable developers are conventional, alkaline, photographic developing solutions useful for standard direct positive emulsions in the absence of the novel fogging agents and their combination with other ingredients. While the silver halide system used in this invention is generally silver chlorobromide, other types, e.g., silver chloride, silver iodobromide, silver iodochloride and silver iodobromochloride may be used with the metalloborane compounds.

Among the metalloboranes which have been found useful as chemical fogging agents in this invention are the metalloboranes, metallothiaboranes and the metallocarboranes, representative examples of which are shown in the following list.

## COMPOUND FORMULA





The general method of preparation of these metalloboranes is described in Polyhedral Boranes by Earl L. Muetterties and Walter H. Knoth, published by Marcel Dekker, Inc. New York and related bibliographic references made of record in that publication.

#### DESCRIPTION OF THE PREFERRED EMBODIMENTS

For most efficient fogging action it is preferred that the metalloborane compounds be added to the silver halide emulsion after it has been made, ripened and washed to remove excess soluble salts resulting from the formation of the silver halides. Conveniently, the metalloborane compounds are added just prior to or during the digestion or "after-ripening" period. The pH of the emulsion is adjusted between 3.0 and 9.0 and preferably between 3.0 and 7.0 and maintained at a preselected level in this range during the digestion period. After digestion, the pH is adjusted to the desired coating pH and the conventional coating aids are added. Coating aids such as saponin, sodium salts of polyether sulfonates, alkyl sulfonates, cetyl betaine etc. can be utilized. The emulsion is then coated and dried in a manner well known to those skilled in the manufacture of photographic silver halide emulsion coated elements.

The sensitometric characteristics of the directpositive emulsions may be determined by exposing strips of elements coated with the emulsions in an intensity scale sensitometer (described on page 616, Mees, The Theory of the Photographic Process, Macmillan Company, New York (1942) using a suitable step wedge and light intensity depending upon the inherent speed of the emulsion. Direct positives are, of course, tailored to meet certain needs in the industry and are manufactured accordingly. After exposure in the sensitometer, the strips are developed in suitable developers as shown below, immersed in a shortstop bath and fixed in a conventional fixer, washed and dried.

In evaluation of the processed strips, the toe of the characteristic curve is equal to the number of steps between density 0.25 and density 0.01. Maximum density ( $D_{max}$ ) is the highest density value obtained on the image of the step wedge. The speed of a typical low speed commercial direct positive in terms of  $100/\text{E} \times 10^{-6}$  is about 103 and the conventional material has a maximum density of about 3.5.

The invention will now be illustrated in and by the following examples:

#### EXAMPLE I

A direct positive emulsion was made in the following manner. To acidified aqueous solution of gelatin containing 1 mole of potassium chloride and  $6.9 \times 10^{-5}$  mole of rhodium trichloride, there was rapidly added 1 mole of silver nitrate in aqueous solution. To the resulting mixture there was added 0.4 mole of potassium bromide in aqueous solution and the resulting emulsion was then ripened by heating for 10 minutes at 160°F. A second portion of 0.6 mole of potassium bromide was added and the emulsion was further ripened for 10 minutes at 160°F.

The resulting emulsion was cooled, coagulated, washed and redispersed in the manner disclosed in Mende, U.S. Pat. No. 2,772,165, issued Nov. 27, 1956.

To the redispersed emulsion there was added bulking gelatin and the pH was adjusted to 7.0 and portions of the emulsion were heated to 130°F during which the borane compound  $\text{CsB}_9\text{H}_{12}\text{S}$  and metalloboranes were added to the portions as indicated in the following table. The emulsions were digested for 60 minutes at 130°F. The borane compound  $\text{CsB}_9\text{H}_{12}\text{S}$  is disclosed and claimed in Assignee's Bigelow U.S. Ser. No. 62,650 filed Aug. 10, 1970 and was used here as a control sample. (It is not a metalloborane but a metal salt of a thiaborane.) After digestion, the emulsion was cooled to 95°F, the wetting agent, saponin, was added and the viscosity was suitably adjusted and the emulsion was coated on a photographic quality film support and dried in a conventional manner. The sensitometric strips were exposed in the above described sensitometer using a No. 3 lamp, SQRTZ Ser. No. 8876418 for 16 seconds. The strips were developed in the two following developers, 3 minutes in Developer I and 1½ minutes in Developer II.

| Developer I (High Contrast Type) |      |       |
|----------------------------------|------|-------|
| Water                            | 500  | ml    |
| Sodium Sulfite (anh.)            | 30.0 | g     |
| Paraformaldehyde                 | 7.5  | g     |
| Potassium metabisulfite          | 2.5  | g     |
| Boric Acid (crystals)            | 7.5  | g     |
| Hydroquinone                     | 22.5 | g     |
| Potassium Bromide                | 1.5  | g     |
| Water to make                    | 1.0  | liter |

| Developer II (Continuous Tone Type) |      |       |
|-------------------------------------|------|-------|
| Water                               | 500  | ml    |
| N-methyl-p-aminophenol (Metol)      | 1.0  | g     |
| Sodium Sulfate (anh.)               | 15.0 | g     |
| Hydroquinone                        | 4.0  | g     |
| Sodium Carbonate (monohydrate)      | 26.9 | g     |
| Potassium bromide                   | 0.6  | g     |
| Benzotriazole                       | 0.1  | g     |
| Water to make                       | 1.0  | liter |

Sensitometric evaluation adduced the following data:

TABLE I

| Strip No. | $4 \times 10^{-6}$ mole per 1.5 moles Ag halide                                             | Dev. | Speed                         | Dmax | Toe | Fog  |
|-----------|---------------------------------------------------------------------------------------------|------|-------------------------------|------|-----|------|
| 1         | Borane Compound<br>$[(p\text{-tolyl})_3\text{P}]_4\text{AgB}_{11}\text{H}_{14}$             | I    | $100/\text{E} \times 10^{-6}$ | 6.0+ |     | 1.56 |
| 2         | $\text{Cs}[\text{B}_{10}\text{H}_{10}\text{S}_2\text{Co}]$                                  | II   |                               | 6.22 |     | 3.73 |
| 3         | $\text{B}_{10}\text{SH}_{10}\text{Re}(\text{CO})_3$                                         | II   | 20,000                        | .89  | 2.6 | .16  |
| 4         | $[(\text{C}_2\text{H}_5)_3\text{P}]_2\text{Pt}(\text{H})\text{B}_{10}\text{H}_{10}\text{S}$ | II   | 110,000                       | .51  | 6.7 | .06  |
| 5         | $[(\text{C}_2\text{H}_5)_3\text{P}]_2\text{PtB}_{10}\text{H}_{12}$                          | II   |                               | 6.0+ |     | .84  |
| 6         | $[(\text{C}_2\text{H}_5)_3\text{P}]_2\text{PtB}_3\text{H}_7$                                | II   |                               | 4.0+ |     | .24  |
| 7         | do.                                                                                         | I    |                               | 4.0+ |     | .23  |
| 8         | $2.4 \times 10^{-6}$ mole/<br>1.5 mole AgHal                                                | II   | 12,300                        | 3.49 |     | .00  |
|           | $\text{CsB}_9\text{H}_{12}\text{S}$ (Control)                                               |      |                               |      |     |      |

Example I was repeated except that hydrochloroauric acid ( $\text{HAuCl}_4$ ) was added to some portions and also the cesium salt of thiaborane ( $\text{CsB}_9\text{H}_{12}\text{S}$ ) was added with the metalloborane compound as indicated in the following table.

It is apparent that an increase in digestion time produces more than twice the density without appreciably affecting fog.

While some of the metalloboranes are less effective than others as chemical fogging agents, in general they

TABLE II

| Fogging Agent Variation |                                    |                                  |                                                                            |      |         |      |     |      |
|-------------------------|------------------------------------|----------------------------------|----------------------------------------------------------------------------|------|---------|------|-----|------|
| Strip No.               | Mole/1.5 Moles<br>$\text{HAuCl}_4$ | Mole/1.5 Moles<br>$\text{AgHal}$ | 4 $\times 10^{-6}$ Mole/<br>1.5 Moles $\text{AgHal}$ .<br>Metalloborane    | Dev. | Speed   | Dmax | Toe | Fog  |
| 1                       |                                    |                                  | $\text{Cs}(\text{B}_{10}\text{H}_{10}\text{CH})_2\text{Fe}$                | II   | —       | 0.0  | —   | —    |
| 2                       | $3.7 \times 10^{-5}$               |                                  |                                                                            |      | 12,000  | 5.68 | 1.2 | 0.10 |
| 3                       |                                    |                                  | $[(\text{p-tolyl})_3\text{P}]_4$<br>$\text{AgB}_9\text{H}_{14}$            | II   |         | .14  | —   | .01  |
| 4                       | $3.7 \times 10^{-5}$               |                                  | do.                                                                        | II   |         | 6.0+ | —   | .16  |
| 5                       |                                    | $4 \times 10^{-8}$               | $\text{Cs}(\text{B}_{10}\text{H}_{10}\text{S})_2\text{Co}$                 | I    | 902,000 | .93  | 5.6 | .00  |
| 6                       |                                    | do.                              | do.                                                                        | II   | 80,000  | 3.88 | 6.1 | .08  |
| 7                       |                                    |                                  | $\text{Cs}_2(\text{B}_{10}\text{H}_{10}\text{CNH}_2)_2\text{Ni}$           | II   |         | 0.0  | —   | —    |
| 8                       | $3.7 \times 10^{-5}$               |                                  | do.                                                                        | II   |         | .14  | —   | —    |
| 9                       |                                    |                                  | $(\text{B}_{10}\text{H}_{10}\text{CNH}_2)_2\text{Ni}$                      | II   |         | 0.0  | —   | —    |
| 10                      | $3.7 \times 10^{-5}$               |                                  |                                                                            | II   | 330,000 | 1.07 | 6.8 | 0.2  |
| 11                      |                                    |                                  | $[(\text{C}_2\text{H}_5)_3\text{P}]_2\text{PtB}_{10}\text{H}_{10}\text{S}$ | II   |         | 0.0  | —   | —    |
| 12                      | $3.7 \times 10^{-5}$               |                                  | do.                                                                        | II   | 340,000 | 1.47 | 5.9 | 0.0  |
| 13                      |                                    | $2.66 \times 10^{-7}$            | Control                                                                    | II   | —       | —    | —   | —    |
| 14                      | $3.7 \times 10^{-5}$               | $4 \times 10^{-8}$               | Control                                                                    | II   | 754,000 | .87  | 8.1 | 0.0  |
| 15                      | $4.95 \times 10^{-5}$              | $2.66 \times 10^{-7}$            | Control                                                                    | II   | 280,000 | 1.37 | —   | .05  |

## EXAMPLE III

Example I was repeated using the metalloborane,  $\text{Cs}(\text{B}_{10}\text{H}_{10}\text{S})_2\text{Co}$  alone and in combination with hydrochloroauric acid ( $\text{HAuCl}_4$ ) and using the borane compound,  $\text{CsB}_9\text{H}_{12}\text{S}$  as a control as indicated in the following table:

are capable of producing extremely fast direct positive elements. The elements of this invention, as shown in the examples, may be developed in any standard developing solution either of the continuous tone type or the high contrast lithographic type using standard techniques. Variations in the developing solution will have

TABLE III

| Strip No. | Mole/1.5 Mole<br>$\text{AgHal}$                            | Mole/1.5 mole<br>$\text{AgHal}$ | Dev. | Speed     | Dmax | Toe  | Fog |
|-----------|------------------------------------------------------------|---------------------------------|------|-----------|------|------|-----|
|           | $\text{Cs}(\text{B}_{10}\text{H}_{10}\text{S})_2\text{Co}$ | $\text{HAuCl}_4$                |      |           |      |      |     |
| 1         | $4 \times 10^{-6}$                                         | 0                               | I    | 16,000    | 2.21 | 3    | .06 |
| 2         | do.                                                        | 0                               | II   | 12,900    | 2.51 | 2.18 | .08 |
| 3         | $4 \times 10^{-7}$                                         | 0                               | I    | —         | 0.0  | —    | —   |
| 4         | do.                                                        | 0                               | II   | —         | 0.0  | —    | —   |
| 5         | $4 \times 10^{-6}$                                         | $3.72 \times 10^{-5}$           | I    | —         | 3.01 | —    | .30 |
| 6         | do.                                                        | do.                             | II   | —         | 2.83 | —    | .30 |
| 7         | $4 \times 10^{-7}$                                         | do.                             | I    | 69,700    | 2.71 | 5.22 | .00 |
| 8         | do.                                                        | do.                             | II   | 72,400    | 2.63 | 5.33 | .00 |
| 9         | $4 \times 10^{-8}$                                         | do.                             | I    | —         | .17  | —    | —   |
| 10        | do.                                                        | do.                             | II   | 1,020,000 | .49  | 9.0  | .00 |
| 11        | $4 \times 10^{-9}$                                         | do.                             | I    | —         | 0.0  | —    | —   |
| 12        | do.                                                        | do.                             | II   | —         | 0.0  | —    | —   |
| 13        | $4 \times 10^{-6}$                                         | do.                             | I    | —         | .19  | —    | —   |
| 14        | $\text{CsB}_9\text{H}_{12}\text{S}$<br>(control)           | do.                             | II   | 947,000   | .49  | 8.75 | .00 |

It will be apparent that the presence of the gold compound produces an effect with an amount of metalloborane which does not occur with the use of the metalloborane alone.

## EXAMPLE IV

Example I was repeated except that the digestion time was varied as indicated in the table and  $3.72 \times 10^{-5}$  mole hydrochloroauric acid per 1.5 moles of silver halide was used with the metalloborane compounds.

much the same effect as it would in developing nonreversal emulsions. No pre-exposure operations or auxiliary processing procedures are necessary or desired in using the novel elements of this invention. It is also unnecessary to utilize stain producing nonsensitizing dyes or other desensitizing compounds in the emulsion. The metalloboranes are far superior to formaldehyde, the principle fogging agent of the prior art, because the metalloboranes do not have a hardening effect on the gelatin layer.

TABLE IV

| Metalloborane |                                                                                     |                          |           |      |           |      |      |     |
|---------------|-------------------------------------------------------------------------------------|--------------------------|-----------|------|-----------|------|------|-----|
| Strip No.     | Formulae                                                                            | Mole per 1.5 Moles AgHal | Dig. Time | Dev. | Speed     | Dmax | Toe  | Fog |
| 4             | do.                                                                                 | do.                      | do.       | II   | 2,090,000 | .31  | 11.0 | .00 |
| 5             | do.                                                                                 | 4×10 <sup>-6</sup>       | do.       | I    | —         | .01  | —    | .00 |
| 6             | do.                                                                                 | do.                      | do.       | II   | —         | .05  | —    | .00 |
| 7             | Cs <sub>2</sub> H <sub>12</sub> S(control)                                          | do.                      | do.       | I    | 947,000   | .47  | 8.75 | .00 |
| 8             | do.                                                                                 | do.                      | do.       | II   | 597,000   | .71  | 7.36 | .00 |
| 9             | Cs <sub>2</sub> (B <sub>10</sub> H <sub>10</sub> CNH <sub>2</sub> ) <sub>2</sub> Ni | 1.5×10 <sup>-5</sup>     | 2 hrs.    | I    | 102,000   | 2.75 | 5.26 | .01 |
| 10            | do.                                                                                 | do.                      | do.       | II   | 85,000    | 2.58 | 5.78 | .01 |
| 11            | do.                                                                                 | 8×10 <sup>-6</sup>       | do.       | I    | 313,000   | .97  | 5.64 | .00 |
| 12            | do.                                                                                 | do.                      | do.       | II   | 217,500   | 1.25 | 4.55 | .00 |
| 13            | do.                                                                                 | 4×10 <sup>-6</sup>       | do.       | I    | —         | .15  | —    | .00 |
| 14            | do.                                                                                 | do.                      | do.       | II   | 1,450,000 | .37  | 10.0 | .00 |
| 15            | Cs <sub>2</sub> H <sub>12</sub> S(control)                                          | do.                      | do.       | I    | 497,000   | .92  | 6.9  | .00 |
| 16            | do.                                                                                 | do.                      | do.       | II   | 271,000   | 1.50 | 5.23 | .00 |

The silver halide emulsions of this invention can be made with any of the macromolecular, water-permeable colloids known to be suitable for the purpose of acting as a colloid carrier for silver halide grains. In addition to gelatin, there may be used polyvinyl alcohol and its derivatives, e.g., partially polyvinyl acetates, ethers and acetals, hydrolyzed interpolymers of vinyl acetate and unsaturated addition polymerizable compounds such as maleic anhydride, acrylic and methacrylic acid esters, poly-N-vinylactams, polysaccharides, e.g., dextran, dextrin, etc., the hydrophilic copolymers disclosed in Shacklett, U.S. Pat. No. 2,833,650, hydrophilic cellulose ethers and esters, and acrylamide polymers. Mixtures of these binders can also be used as well as water-permeable binding agents containing dispersed polymerized vinyl compounds such as those disclosed in Nottorf, U.S. Pat. No. 3,142,568 issued July 28, 1964.

The emulsions of this invention may be coated on any suitable support including photographic quality paper and transparent film. For example, the cellulosic support, e.g., cellulose acetate, cellulose triacetate, cellulose mixed esters, etc., may be used. Polymerized vinyl compounds, e.g., copolymerized vinyl acetate and vinyl chloride, polystyrene and polymerized acrylates may also be mentioned. The film formed from the polyesters made according to the teachings of Alles, U.S. Pat. No. 2,779,684 and the patents referred to in the specification of that patent may be used. Other suitable supports are the polyethylene terephthalate/isophthalates of British Patent No. 766,290 and Canadian Patent 562,672 and those obtainable by condensing terephthalic acid and dimethyl terephthalate with propylene glycol, dimethylene glycol, tetramethylene glycol or cyclohexane-1,4-dimethanol(hexahydro-p-xylene alcohol). The films of Bauer et al., U.S. Pat. No. 3,059,543 may also be used. The above polyester films are particularly suitable because of their dimensional stability. The emulsions are generally coated on the supports to

give a silicone nitrate coating weight equivalent to about 700 mg/ft<sup>2</sup>.

Many metalloborane compounds other than those referred to above can be used as chemical fogging agents for the direct positive photographic elements of this invention.

25 25 What is claimed is:

1. A direct-positive, colloid-silver halide emulsion containing a fogging amount of a borane selected from the group consisting of metalloboranes, metallothiaboranes and metallocarbonanes, said borane having three or eight to 11 boron atoms and containing in its structure at least one metal selected from the group consisting of platinum, nickel, cobalt, rhenium, iron and silver.
2. An emulsion according to claim 1 having a pH below about 9.0.
3. An emulsion according to claim 1 wherein the amount ranges from 10<sup>-8</sup> to 10<sup>-4</sup> mole per 1.5 moles of silver.
4. An emulsion according to claim 3 containing a salt of rhodium or iridium.
5. An emulsion according to claim 3 wherein the silver halide is silver chloride.
6. An emulsion according to claim 3 wherein the silver halide is silver chlorobromide.
- 45 45 7. An emulsion according to claim 3 wherein said colloid is gelatin.
8. A direct-positive photographic element comprising a sheet support bearing a layer of a silver halide emulsion as defined in claim 3.
- 50 9. An element according to claim 8, wherein the silver halide is silver chloride.
10. An element according to claim 8 wherein the silver halide is silver chlorobromide.
- 55 11. An element according to claim 8 containing a salt of rhodium or iridium.

\* \* \* \* \*